

# United States Patent Office

3,808,111

Patented Apr. 30, 1974

1

3,808,111

## DRY LUBRICANT COATED ARTICLE

Ralph J. Hovey, 1N600 Glenrise Ave., Glen Ellyn, Ill. 60137, and Afsar A. Khan, 921 Cedar Ave., Elmhurst, Ill. 60126

No Drawing. Continuation of application Ser. No. 879,551, Mar. 4, 1970, which is a continuation-in-part of application Ser. No. 832,476, June 11, 1969, now Patent No. 3,567,597, which in turn is a division of abandoned application Ser. No. 520,360, Jan. 3, 1966. This application Jan. 26, 1973, Ser. No. 327,549

Int. Cl. C23b 9/02, 11/02

U.S. CL. 204—56 R

12 Claims

## ABSTRACT OF THE DISCLOSURE

A member of a base metal such as aluminum, magnesium, titanium or tin is electrolytically anodized while simultaneously electrophoretically depositing solid lubricant particles of colloidal size, so as to produce a lubricating coating tightly bonded to the surface of the member with the particles being distributed throughout the thickness of an oxide on the surface and being locked in place within randomly oriented interstices within the oxide. Preferably, the solid lubricant particles are of Teflon and the base metal is aluminum, but various other solid lubricant particles and base metals may be used.

This is a continuation of application Ser. No. 879,551, filed Mar. 4, 1970, which is a continuation-in-part of application Ser. No. 832,476, filed June 11, 1969 and issued as U.S. 3,567,597, which is a division of, and which was copending with, application Ser. No. 520,360, filed Jan. 3, 1966, now abandoned.

The invention relates to a dry lubricant coated article. More particularly the invention relates to incorporating particles of a solid lubricant into the anodized surface of a metal to form a dry lubricant coating.

An object of the invention is to provide a strongly adherent dry lubricant coating.

A further object is to provide a method of quickly and economically producing an anodized metal surface having superior lubricating qualities to that of an ordinary anodized surface.

Another object is to provide a method of producing a dry lubricant comprising an anodized metal surface containing particles of a fluorocarbon polymer.

Other objects and advantages of the invention will become apparent as the following detailed description progresses.

In accordance with this invention an anodizable metal such as aluminum, titanium, tin or magnesium is electrolytically anodized as is well known to the art and while the anodization is taking place there is electrophoretically deposited on the metal particles of a solid lubricant. This simultaneous electrolytic growth of oxide and electrophoretic deposition of a lubricating media is accomplished by incorporating in the electrolyte being used for the anodization a negatively charged particle of a solid lubricant. Thus, when the metal is made the anode and oxidation is taking place by electrolysis at the anode, the negatively charged particles of solid lubricant will migrate by means of the electric current induced in the bath to the anode and will be commingled (mingled) with the oxide coating during its formation. By this procedure the particles are substantially uniformly distributed throughout the thickness of said oxide and are locked in place with randomly oriented interstices within said oxide to form with the oxide a lubricating coating tightly bonded to the surface of the base metal. This gives an extremely adherent low coefficient of friction coating useful as a bearing surface and for other uses of dry lubricants.

2

The thickness of the coating is a function of the treatment time. Suitable coatings have been made with .001 inch thickness and as thick as .005 inch, but lesser and greater thicknesses can be attained.

5 The preferred metals used for simultaneous anodization and electrophoretic deposition of solid particles are aluminum, titanium, magnesium and the alloys containing a major portion of such metals. The oxide coating produced is better suited for the commingling (mingling) with solid lubricants such as fluorocarbon polymers, and gives a superior lubricating coat than produced by anodizing tin.

All types of solid lubricant particles which normally have or which can be made to have a negative charge 15 may be used. Thus particles of molybdenum disulphide, alumina-tungsten disulphide, polyethylene, and fluorocarbon polymers can be used. For lubricating purposes the fluorocarbon polymers are preferred, particularly the completely fluorinated fluorocarbon polymers, of which the 20 best appears to be tetrafluoroethylene. The suitable fluorocarbon polymers include polytetrafluoroethylene, polyhexafluoropropylene, polychlorotrifluoroethylene, polyvinylidene fluoride, polyvinyl fluoride, tetrafluoroethylene-hexafluoropropylene copolymer, vinylidene fluoride-hexafluoropropylene copolymer, poly 1,1,1-trifluoropropyl-methyldichlorosilane polymer, fluorosilicone elastomers, polyfluoroaniline, and copolymers of tetrafluoroethylene and trifluoromethane. The preferred completely fluorinated fluorocarbon from the point of view of coefficient of friction and all around value, is polytetrafluoroethylene. This material under the trademark Teflon is commercially available as negatively charged colloidal particles dispersed in an aqueous liquid.

The following example illustrates the invention:

## EXAMPLE I

An aluminum sheet is made the anode. The cathode is lead or stainless steel. The electrolyte consists of sulfuric acid (10 fluid ounces per gallon), oxalic acid (2 ounces per gallon), an aqueous suspension of negative charged colloidal particles of polytetrafluoroethylene containing 0.5 percent by weight TFE (Teflon suspension No. 3170) acidulated with 5 percent sulfuric acid, the ingredients being merged in water to a volume of two gallons. 40 The electrolyte was contained in a glass tank and maintained at a temperature of 25°–95° F. during the operation. The current density used was 10–36 amperes per square foot. The voltage was 10–75 volts. Vigorous agitation of the electrolyte was maintained. The time of operation was 15 to 60 minutes.

The coated plate produced by the above example had a coating of mixed aluminum oxide and particles of polytetrafluoroethylene of 0.002–0.0025 inch thickness.

Substantially the same results as with the above example 55 may be obtained with the other fluorocarbon polymers above mentioned using similar procedure and conditions as in Example I. With particles of molybdenum disulphide and other metal sulfides a suitable commingled (mingled) coating was also obtained by substituting a molybdenum disulphide aqueous dispersion for the Teflon dispersion and otherwise keeping the conditions the same, although modification of the procedure to obtain better anodic deposition of the molybdenum disulphide could be carried out in accordance with procedures known to 60 the art without interfering with the simultaneous anodization. Polyethylene does not give as satisfactory lubricating properties as the fluorocarbon polymers but can also be electrophoretically deposited during electro anodization using the procedure and condition of Example I.

The use of negatively charged colloidal particles as above disclosed for the electrophoretic deposition gives particles of colloidal size commingled (mingled) with the

oxide of the anodized metal base. By following the procedures of the example there is obtained an article comprising a member of a base metal such as aluminum, an oxide of said base metal and of substantial thickness anodized on a surface of said member, and solid lubricant particles of colloidal size (.001-.5 micron diameter) mingled with said oxide, said particles being substantially uniformly distributed throughout the thickness of said oxide and being locked in place within randomly oriented interstices within said oxide to form with said oxide a lubricating coating tightly bonded to the surface of the base metal.

The resultant oxide has at least a portion of the particle of lubricant deposited in some interstices below the bearing or outer surface of the oxide with these interstices not normally accessible by direct treatment of the bearing surface with similarly sized particles of the lubricant.

The above procedure of Example I may be suitable for other anodizable metals including titanium and magnesium.

What is claimed is:

- An article comprising a member of a base metal, an oxide of said base metal and of substantial thickness anodized on a surface of said member and including an upper surface opposite said member, and solid lubricant particles mingled with said oxide, said particles being substantially uniformly distributed throughout the thickness of said oxide and being locked in place within randomly oriented interstices within said oxide to form with said oxide a lubricating coating tightly bonded to said surface, at least a portion of said particles being deposited below said upper surface during formation of said oxide by anodizing.
- An article as defined in claim 1 wherein the solid lubricant particles are of colloidal size.
- An article as defined in claim 2 wherein said base metal is aluminum.
- An article as defined in claim 2, wherein said base metal is magnesium.
- An article as defined in claim 2 wherein said base metal is titanium.
- An article as defined in claim 2 wherein said solid lubricant particles are particles of a fluorocarbon polymer.

7. An article as defined in claim 2 wherein said solid lubricant particles are particles of molybdenum sulphide.

8. The article of claim 6 wherein the base metal is aluminum and wherein the particles are of polytetrafluoroethylene.

9. An article as defined in claim 8 wherein said solid lubricant particles are electrophoretically deposited and mingled with said oxide during formation of said oxide on said surface of said member, and a major portion of said particles being in the range of 0.001-0.5 micron in diameter.

10. An article comprising a member of a base metal, an oxide of said base metal and of substantial thickness anodized on a surface of said member, and including an upper surface opposite said member, and solid lubricant particles mingled with said oxide, said particles being substantially distributed throughout said oxide and being locked in place within randomly oriented interstices within said oxide to form with said oxide a lubricating coating tightly bonded to said surface, at least a portion of said particles being electrophoretically deposited below said upper surface during formation of said oxide by anodizing.

11. An article as defined in claim 10 wherein the base metal is aluminum and the particles are of polytetrafluoroethylene and are of colloidal size.

12. An article as defined in claim 11 wherein said particles are deposited in an electroplating system comprising an anode of said base metal, a cathode, and an electrolyte containing said particles with a negative charge.

#### References Cited

##### UNITED STATES PATENTS

|           |         |               |          |
|-----------|---------|---------------|----------|
| 3,716,348 | 2/1973  | Perkins       | 117-75   |
| 3,711,313 | 1/1973  | Nagand et al. | 117-75   |
| 3,438,789 | 4/1969  | Weiss et al.  | 204-56 R |
| 3,271,653 | 9/1966  | Wolf          | 117-75   |
| 3,211,325 | 10/1965 | Wisnicki      | 220-64   |
| 3,052,590 | 9/1962  | Maros et al.  | 117-75   |

JOHN H. MACK, Primary Examiner

R. L. ANDREWS, Assistant Examiner

U.S. CL. X.R.

204-58; 117-75